

E. H. STEEDMAN,  
PROCESS FOR FORMING HOLLOW FORGINGS,  
APPLICATION FILED MAR. 31, 1916.

1,212,120.

Patented Jan. 9, 1917.

Fig. 1.



Fig. 2.



Fig. 3.



Fig. 4.



Inventor,  
E. H. Steedman.  
By Bakewell & Howes, Patents.

# UNITED STATES PATENT OFFICE.

EDWIN H. STEEDMAN, OF ST. LOUIS, MISSOURI.

## PROCESS FOR FORMING HOLLOW FORGINGS.

1,212,120.

Specification of Letters Patent.

Patented Jan. 9, 1917.

Application filed March 31, 1916. Serial No. 88,054.

*To all whom it may concern:*  
Be it known that I, EDWIN H. STEEDMAN, a citizen of the United States, residing at St. Louis, Missouri, have invented a certain 5 new and useful Improvement in Processes for Forming Hollow Forgings, of which the following is a full, clear, and exact description, such as will enable others skilled in the art to which it appertains to make and 10 use the same.

This invention relates to a novel process for making hollow forgings.

Heretofore it was practically impossible to produce uniformly accurate forgings in 15 making hollow forgings by piercing a hole or cavity in a billet or metal blank, on account of the tendency of the piercing punch to deflect from a straight line when operating on some billets or to be improperly positioned with relation to the outer surface 20 of the forgings when operating on other billets. One method that has been tried to overcome the objections above referred to is to arrange a guide adjacent the open end 25 of the die, so as to try to start the piercing punch at the center of the die, but commercially this is not possible, on account of the piercing punch becoming very hot when in use and on account of the fact that it is not 30 possible to make a guide that will compensate for the rapid wear on the end of the piercing punch, and thus guide the piercing punch accurately after it has been in use for 35 a short time. Even when such a guide is used the irregular shape of the end of the piercing punch bearing on the end of the billet has a tendency to force the punch laterally during the first few inches of its travel through the billet. This, of course, 40 springs the piercing punch out of true axial alinement with the die, and as the punch enters farther into the billet, the spring or deflection greatly increases, frequently resulting in bending the piercing punch. As 45 the billet is usually merely dropped into the die and not compressed prior to the piercing operation, there are voids between the outer surface of the billet and the inner surface of the die. Consequently, even 50 though the piercing punch is accurately guided, a thing that is not possible commercially, the unequal resistance caused by the voids on the side of the die cause the punch to travel out of axial alinement with the die as soon as it enters the billet to a reasonable extent.

The main object of my invention is to provide a metal forging process that will insure the production of uniformly accurate hollow forgings having cavities or center 60 openings that are accurately alined and properly positioned.

Another object is to provide a process for making hollow forgings which makes it possible to use a billet or metal blank of 65 irregular form that does not even approximately fit the die, or a billet or metal blank in which the end operated upon by the piercing punch is irregular in shape, such as a sheared billet whose end has not been 70 squared after coming from the rolls. To this end I have devised a metal forging process in which the billet or blank being operated on is subjected to such treatment prior to the piercing operation that it will 75 accurately position and guide the piercing punch that forms the cavity or center opening in the billet.

Briefly described, my process consists in compressing a heated billet or metal blank 80 and forming a depression in said compressed portion, either in one operation or in successive operations, and thereafter forming a cavity, hole or opening in the billet by means of a piercing punch, or other suitable member which is guided by the metal surrounding the depression in the compressed portion of the billet, the outer surface of the billet being preferably shaped simultaneously with the operation of forming the 85 cavity in same. Any suitable apparatus may be used in practicing my process, and while I have herein illustrated my process used for making a hollow forging provided with a closed end, I wish it to be understood 90 that my invention is applicable to a forging process in which a hole is punched through a billet, so as to form a tubular-shaped article.

Figure 1 of the drawings is a vertical sectional view of an apparatus that may be used in practising my process to compress the billet or blank and form a depression in the compressed portion of same, showing the billet prior to the compressing operation. Fig. 2 is a vertical sectional view of said apparatus, showing the billet after it has been compressed and provided with a depression, the plunger in said apparatus being guided by a member arranged adjacent the open end of the die. Fig. 3 is a vertical sectional view, illustrating the piercing punch enter-

ing the depression in the billet, preparatory to the operation of forming the cavity in the billet; and Fig. 4 is a sectional view, illustrating the billet after the piercing operation has been completed.

Referring to the drawings, 1 designates the billet or metal blank from which the article is to be formed. Said billet is arranged in a die A while in a heated condition, the billet being so shaped and proportioned that it can be dropped into the die A easily, even though the outer surface of the billet is irregular and has slight projections thereon. Thereafter, the billet is compressed 10 and a depression is formed in said compressed portion by means of a forming plunger B provided with a projection B' that is arranged or accurately guided in longitudinal alinement with the center axis of the die 15 A, so that the cavity or center opening in the completed article will be concentric with the outer surface of the article, the projection B' of the forming plunger preferably being of substantially conical shape, although it 20 might be cylindrical, square, or of any desired shape without departing from the spirit of my invention. The die A conforms to the shape of the outer surface of the article being formed, and when the forming 25 plunger B acts on the billet, as shown in Fig. 2, it forms a depression 2 in the upper end of the billet, distorts the metal in the billet and forces the metal in the upper end portion of the billet laterally toward the 30 side walls of the die A, causing the billet to fill the die sufficiently to offer an equal resistance on all sides to the piercing punch or member used in the succeeding operation. While I prefer to form a depression in the 35 billet and compress the metal into the die to the desired extent in one operation, it will, of course, be obvious that the billet could be compressed and a depression formed in said compressed portion by two separate and 40 distinct operations. The forming plunger B is guided accurately, either by the upper end portion of the die A, or by a suitable guiding member A', shown at Fig. 2, arranged adjacent the open end of the die A, 45 so as to prevent said forming plunger from being forced sidewise when it strikes a billet with an irregular upper end, as shown in Fig. 1, it being an easy matter to secure a good mechanical guide for the forming plunger B, on account of the fact that said 50 plunger does not become heated to any appreciable extent and because the large lateral surface of the plunger can be readily lubricated.

The final step in the forging operation 55 consists in forming a cavity or hole in the billet and distorting the metal sufficiently to cause the outer surface of the billet to conform accurately to the shape of the die A, 60 this final step being preferably effected by

a piercing punch or member C which is forced into the metal contained by the die A after the forming plunger B has been withdrawn. When the piercing punch C moves toward the die A, the end of said 70 punch, which is tapered or substantially conical-shaped, enters the depression 2 in the upper end of the billet, thus causing the punch C to be centered accurately with relation to the die A. In view of the fact 75 that the metal in the upper end portion of the billet is compressed until it practically fills the upper portion of the die A and is of substantially equal density surrounding the depression 2, the upper end portion of 80 the billet will offer sufficient resistance on all sides to the punch C, to hold said punch straight when it starts to distort the metal in the billet. As the punch C continues to move through the billet, it is held perfectly 85 straight and is prevented from deflecting from a straight line by means of the compressed metal surrounding the depression 2 in the billet and by the metal that is compressed progressively and equally as the 90 punch C travels through the billet. The result is that the completed forging will be commercially accurate, as the metal is distributed evenly throughout all portions of 95 same, and the center cavity is concentric with the outside of the forging.

As previously stated, any suitable apparatus may be used in practising my process, and while I have referred to the forming plunger B and the punch C as being moved 100 toward the die A, it will of course be obvious that the die in which the billet is arranged could be moved with relation to the members that act upon the billet.

The process above described makes it 105 possible to produce hollow forgings of uniform shape and size in which the center openings are accurately formed and in which the metal in all portions of the side walls of each article is of uniform density. 110

Having thus described my invention, what I claim, and desire to secure by Letters Patent, is:

1. A process for forming a hollow forging, characterized by forming a depression or 115 recess in a billet, and also compressing the metal surrounding said depression prior to the operation of forming a cavity or center opening in the billet.

2. A process for forming a hollow forging, characterized by forming a depression or recess in a billet and also subjecting the billet to longitudinal pressure in a die so as to compress the metal surrounding said depression in the billet and thus cause the 120 metal to substantially fill the adjacent portion of the die, prior to the operation of forming a cavity or center opening in the billet.

3. A process for forming a hollow article, 130

- which consists in compressing a billet or metal blank in a die and also simultaneously forming a depression in said billet by a member that exerts longitudinal pressure on the billet, and thereafter forming a cavity or opening in the billet by means of a member that is centered by the depression in the billet and guided by the compressed metal in the billet that surrounds said depression. 10
4. A process for forming a hollow forging, which consists in forming a depression in a heated billet or metal blank and also compressing the metal around said depression so that it is of substantially uniform density, and thereafter forging said billet into the shape of a hollow article by a member that enters the depression formed in the billet during the first part of the forging operation. 15
5. A process for forming a hollow forging, which consists in forming a depression in a heated billet arranged in a die and also compressing the billet so as to fill the die to the desired extent around said depression, and thereafter forging said billet into a hollow article by a member that enters the depression in the billet during the first part of the forging operation.
6. A process for forming a hollow forging, which consists in arranging a billet or metal blank in a die, subjecting the billet to endwise pressure so as to compress one end portion of same forming a depression in the compressed portion of said billet concentric with the side walls of said die, and thereafter forming a cavity or center opening in the billet in a single operation by means of a piercing punch that is centered and guided by the depression in the billet. 40
7. A process for forming a hollow forging, which consists in compressing a billet or metal blank in a die and also forming a depression in said billet concentric with the side walls of said die, and thereafter forming a cavity or center opening in the billet by means of a piercing punch that is centered by said depression and guided by the metal in the billet surrounding said depression. 45
8. A process for forming a hollow forging, characterized by compressing a billet or metal blank in a die and also simultaneously forming a depression in said billet concentric with the side walls of said die, 50 the billet being compressed to a sufficient extent so that when the piercing punch used in the subsequent operation is started into said depression a substantially equal resistance will be offered on all sides to the 55 piercing punch while it is traveling through the billet to form the center opening or cavity in the billet.

In testimony whereof I hereunto affix my signature in the presence of two witnesses, 60 this twenty-eighth day of March, 1916.

EDWIN H. STEEDMAN.

Witnesses:

W. A. YAEGER,  
A. P. Fox.